

## UNITED STATES PATENT OFFICE

KARL LEO MEISSNER, OF BERLIN, GERMANY

## METHOD OF MANUFACTURING CHEMICALLY-PURE ALUMINUM BY ELECTROLYSIS

No Drawing. Application filed August 1, 1927, Serial No. 210,021, and in Germany December 2, 1926.

In the metallurgical production of aluminum by electrolysis of a mixture of alumina and cryolite there is attained as is known an aluminum of technical purity, which at the most reaches a content of about 99.6% Al. The impurities consist chiefly of iron and silicon.

Only within recent time there has been known a process for obtaining a pure aluminum with an Al content of about 99.8 to 99.9%. This process depends upon the fact that the usual metal aluminum is subjected to a further special electrolytic purification.

According to the process use is made of three layers located one over another, of which the aluminum to be purified forms the lowermost layer as anode layer, while the purified aluminum presents the uppermost layer as cathode layer. Both layers are separated from one another by means of the electrolyte. In order to maintain the necessary difference in specific gravities of the three layers, a heavier addition of some kind must be given not only to the electrolyte but also to the anode layer. For this purpose the aluminum to be purified has been alloyed with copper. This had for a result however that the pure aluminum separating on the cathode contained only small traces of iron and silicon, but instead of it copper as substantial impurification.

The present invention depends upon the fact of employing as anode layer aluminum preliminarily prepared with about 99.8 to 99.9% Al according to the known process already mentioned and further purifying to chemically pure aluminum according to known process. In order to maintain the necessary specific gravity of the anode layer and to enable its deposition as the lowermost layer, in the process according to the present invention copper is not added, which would separate out again in certain quantities in the cathode layer, but instead of this a difficultly oxidizable precious metal of high specific

gravity, as for example gold or platinum or other metals of this group, also, however, silver or nickel.

Thereby it is most favorable to choose a metal of this kind which is not taken up by aluminum in large quantities in solid solution like the copper according to the known process, but which is practically insoluble in solid condition in aluminum. The choice of a metal of specially high specific gravity, as for instance gold or platinum, enables thereby also the amount of addition of this metal to the anode layer for the purpose of increasing the specific gravity to be kept considerably lower than that possible by the addition of copper. By this means there is the possibility further reduced that traces of the alloyed metal separate together with the aluminum on the cathode and thereby again purify the aluminum. Since the addition of precious remains permanently unchanged in the anode layer, and the anode layer is only renewed with preliminary purified aluminum the process by the use of precious metal is not uneconomical.

I claim:

1. The process of manufacturing chemically pure aluminum which consists in passing a current from an anode through the bath to the cathode, where the anode is heavier than the electrolyte and consists of purified aluminum to which has been added a heavy difficultly oxidizable metal.
2. The process of manufacturing chemically pure aluminum which consists in passing a current from an anode through the bath to the cathode, where the anode is heavier than the electrolyte and consists of aluminum preliminarily purified up to from 99.8 to 99.9 per cent to which has been added a heavy difficultly oxidizable metal.
3. The process of manufacturing chemically pure aluminum which consists in passing a current from an anode through the bath to the cathode, where the anode is heavier than

the electrolyte and consists of purified aluminum to which has been added a precious metal.

4. The process of manufacturing chemically pure aluminum which consists in passing a current from an anode through the bath to the cathode, where the anode is heavier than the electrolyte and consists of purified aluminum to which has been added gold.

10 In testimony whereof I affix hereto my signature.

**KARL LEO MEISSNER.**

**15**

**20**

**25**

**30**

**35**

**40**

**45**

**50**

**55**

**60**

**65**